



US012209320B2

(12) **United States Patent**  
**Wakerley et al.**

(10) **Patent No.:** **US 12,209,320 B2**  
(45) **Date of Patent:** **\*Jan. 28, 2025**

(54) **COATED ELECTRONEUTRAL POROUS SEPARATORS FOR OXOCARBON ELECTROLYZERS**

(71) Applicant: **Dioxycle**, Saint Ouen sur Seine (FR)

(72) Inventors: **David Wakerley**, Paris (FR); **Edward Luke Malins**, Bordeaux (FR); **Sarah Lamaison**, Paris (FR); **Renjie Liu**, Paris (FR); **Thomas A. R. Horton**, Paris (FR)

(73) Assignee: **Dioxycle**, Saint Ouen sur Seine (FR)

(\*) Notice: Subject to any disclaimer, the term of this patent is extended or adjusted under 35 U.S.C. 154(b) by 0 days.

This patent is subject to a terminal disclaimer.

(21) Appl. No.: **18/582,903**

(22) Filed: **Feb. 21, 2024**

(65) **Prior Publication Data**

US 2024/0200212 A1 Jun. 20, 2024

**Related U.S. Application Data**

(63) Continuation-in-part of application No. 18/123,353, filed on Mar. 20, 2023, now Pat. No. 12,139,801.  
(Continued)

(51) **Int. Cl.**  
**C25B 13/08** (2006.01)  
**C25B 3/03** (2021.01)  
(Continued)

(52) **U.S. Cl.**  
CPC ..... **C25B 13/02** (2013.01); **C25B 3/03** (2021.01); **C25B 3/25** (2021.01); **C25B 3/26** (2021.01); **C25B 9/19** (2021.01); **C25B 13/08** (2013.01)

(58) **Field of Classification Search**

None

See application file for complete search history.

(56) **References Cited**

**U.S. PATENT DOCUMENTS**

6,287,730 B1 \* 9/2001 Callahan ..... B01D 71/26  
429/246  
8,173,305 B2 5/2012 Holzapfel et al.  
(Continued)

**FOREIGN PATENT DOCUMENTS**

EP 3626858 A1 3/2020  
WO 2023180908 A1 9/2023

**OTHER PUBLICATIONS**

Davis J, Membraneless Electrolyzers for Solar Fuel Production, Columbia University, Doctoral Theses, 2019. (Available at: <https://academiccommons.columbia.edu/doi/10.7916/d8-ypyq-6d71>).

(Continued)

*Primary Examiner* — Wojciech Haske

(74) *Attorney, Agent, or Firm* — Daylight Law, P.C.

(57) **ABSTRACT**

Methods and systems related to oxocarbon electrolyzers are disclosed herein. A disclosed system includes an oxocarbon electrolysis reactor. The reactor includes an aqueous anode area with an oxidation substrate, a gaseous cathode area with an oxocarbon species as a reduction substrate, and an electroneutral separator separating the anode area and the cathode area while allowing ionic migration between the anode area and cathode area. In specific approaches disclosed herein the electroneutral separator is a polymer having a coating, the coating is formed of an aliphatic molecule, and the coating increases a hydrophilicity of the electroneutral separator. In specific approaches disclosed herein, the electroneutral separator is a polymer having a coating, the polymer comprises aliphatic carbon chains, and

(Continued)

100



the coating is an aliphatic carbon chain with one or more hydrophilic functional groups.

**24 Claims, 15 Drawing Sheets**

|              |     |         |                         |
|--------------|-----|---------|-------------------------|
| 10,961,632   | B2  | 3/2021  | Ono et al.              |
| 11,130,723   | B2  | 9/2021  | Kudo et al.             |
| 2008/0257722 | A1  | 10/2008 | Tomba et al.            |
| 2019/0085470 | A1  | 3/2019  | Ono et al.              |
| 2020/0002822 | A1  | 1/2020  | Ono et al.              |
| 2021/0079543 | A1  | 3/2021  | Mikoshiba et al.        |
| 2021/0292926 | A1  | 9/2021  | Ono et al.              |
| 2022/0298655 | A1* | 9/2022  | Kofuji ..... C25B 13/08 |

**Related U.S. Application Data**

(60) Provisional application No. 63/446,321, filed on Feb. 16, 2023, provisional application No. 63/322,639, filed on Mar. 22, 2022.

**(51) Int. Cl.**

|                   |           |
|-------------------|-----------|
| <i>C25B 3/25</i>  | (2021.01) |
| <i>C25B 3/26</i>  | (2021.01) |
| <i>C25B 9/19</i>  | (2021.01) |
| <i>C25B 13/02</i> | (2006.01) |

**(56) References Cited**

## U.S. PATENT DOCUMENTS

|            |    |         |             |
|------------|----|---------|-------------|
| 9,518,329  | B2 | 12/2016 | Wang et al. |
| 10,490,849 | B2 | 11/2019 | Lee et al.  |
| 10,883,180 | B2 | 1/2021  | Ono et al.  |

## OTHER PUBLICATIONS

Final Office Action dated Oct. 20, 2023 from U.S. Appl. No. 18/123,353, 17 pages.

International Search Report and Written Opinion from International Application No. PCT/IB2023/052735 dated Sep. 12, 2023, 9 pages. J. Fang et al. (2018). Journal of Membrane Science vol. 549, p. 332-349.

Lin R, Guo J, Li X, Patel P, Seifitokaldani A. Electrochemical Reactors for CO<sub>2</sub> Conversion. Catalysts. 2020; 10(5):473. (Available at: <https://doi.org/10.3390/catal10050473>).

Non-final Office Action from U.S. Appl. No. 18/123,353 dated Jun. 13, 2023, 11 pages.

Non-Final Office Action dated Mar. 28, 2024 from U.S. Appl. No. 18/123,353, 9 pages.

Notice of Allowance dated Sep. 11, 2024 from U.S. Appl. No. 18/123,353, 9 pages.

\* cited by examiner



FIG. 1



**FIG. 2**  
(Related Art)



FIG. 3



FIG. 4



FIG. 5



FIG. 6



FIG. 7



FIG. 8



FIG. 9



FIG. 10



FIG. 11



FIG. 12



FIG. 13



FIG. 14



FIG. 15

# COATED ELECTRONEUTRAL POROUS SEPARATORS FOR OXOCARBON ELECTROLYZERS

## CROSS REFERENCE TO RELATED APPLICATIONS

This application is a continuation-in-part of U.S. patent application Ser. No. 18/123,353 filed Mar. 20, 2023, which claims the benefit of U.S. Provisional Patent Application No. 63/446,321 filed Feb. 16, 2023, and U.S. Provisional Patent Application No. 63/322,639 filed Mar. 22, 2022, all of which are incorporated by reference herein in their entireties for all purposes.

## BACKGROUND

There is an urgent need to reduce the emissions related to the production of useful fuels and chemicals in our society. Furthermore, there is an urgent need to develop technologies which make the capture or direct valorization of carbon dioxide more economical. Accordingly, technologies that both generate useful fuels and chemicals, while at the same time using carbon dioxide feedstock that would otherwise have been emitted into the atmosphere, are critically important because they both generate useful chemicals without additional emissions and because the economic value of the useful chemicals can offset the cost of carbon dioxide capture and conversion.

A class of technologies that can address the problems outlined in the prior paragraph are oxocarbon electrolyzers. These devices take an oxocarbon as an input and can be used to produce valuable chemicals by valorizing the oxocarbon. Electrolyzers are reactors that operate using a paired reduction and oxidation reaction. The reduction reaction occurs in a cathode area of the reactor and the oxidation reaction occurs in an anode area of the reactor. The two areas are separated by a charged ion exchange membrane. The charged ion exchange membrane allows ions from the reduction and/or oxidation reaction to migrate across the reactor to allow for the reduction and oxidation reactions to take place. The charged ion exchange membranes can be configured to allow facile migration of anions, cations, or both types of charged ions. In addition to providing for ion migration, the ion exchange membranes must be mechanically stable as they serve to physically isolate compartments of the electrolyzer and can also serve as supports for electrodes in either the anode area, the cathode area, or both.

The ion exchange membrane can take the form of one or more charged membranes chosen among anion-exchange membranes (such as, but not limited to, commercial Acmion®, Orion®, Sustainion®, Piperion®, or ionomer anion-exchange membranes), cation-exchange membranes (such as but not limited to Nafion®, Aquivion®, or other commercial membranes), and bipolar membranes (such as, but not limited to, Fumasep® FBM and Xion®). An anion-exchange membrane may be prepared using N-bearing monomers. Anion exchange membranes in oxocarbon electrolyzers are designed to selectively allow anions, such as hydroxide, to migrate from the cathode area to the anode area. Cation exchange membranes in oxocarbon electrolyzers are designed to selectively allow cations to migrate from the anode area to the cathode area. Bipolar membranes include both an anion exchange membrane and a cation exchange membrane with a water dissociation layer between

the two membranes and allow both anions and cations to migrate between the anode area and the cathode area of the electrolyzer.

Charged ion exchange membranes are charged through the implanting of charged chemicals into the material that forms the membrane to facilitate their ability to allow for the migration of ions. Approaches for treating separator material by implanting charged chemicals while maintaining sufficient mechanical stability and other desirable characteristics for separators in electrolysis reactors are expensive which adds significantly to the overall cost of the electrolysis reactor into which they are installed.

## SUMMARY

This disclosure relates to separators used in oxocarbon electrolyzers. In specific embodiments of the invention, an electrolysis reactor includes an anode area and a cathode area with an electroneutral separator separating the anode area and the cathode area. The electroneutral separator can be a membrane, diaphragm, or any separator. The electroneutral separator can be formed by electrically insulative material while being ionically conductive. As such, the separator can allow for ionic migration between the anode area and cathode area while still separating the anode area and the cathode area. The separator can also serve as a support for one or more electrodes in the anode area or cathode area. The separator can be electroneutral in that it is formed entirely of insulative material. The separator can be electroneutral in that no charged chemicals are bound into the electroneutral separator. The incorporation of charged chemicals into a membrane is a costly process that significantly increases the cost of the membrane. As such, using approaches disclosed herein, an electrolysis reactor can thereby provide for migration of ionic species between the anode and cathode while the overall cost of the electrolyzer is greatly reduced. Furthermore, as the amount of incorporated electrical charge and mechanical stability of a traditional membrane are often tradeoffs in the design, approaches disclosed herein exhibit significant benefits in that the separator can be made mechanically sturdy without regard to optimizing for a negatively correlated property.

The use of an electroneutral separator provides significant benefits as compared to other approaches because the cost of fabrication is lower and because the separator is overall more reliable than alternative approaches. The ion conducting membrane in an oxocarbon electrolyzer is one of its major sources of unreliability. The necessity to present both an ion exchange environment and structural stability to the electrode presents a zero-sum game, where increases to the structural stability of the membrane comes at the cost of ion exchange capacity and visa-versa. This makes the production of stable oxocarbon electrolyzer stacks particularly difficult and important. The separator is a critical component and membrane ruptures in one cell may lead to deactivation of the entire unit. The use of charged membranes also prevents the use of high differential pressures across the electrolyzer, due to structural weakness, but these high differential pressures are often desirable to encourage the correct catalytic environment in the system. High differential pressures are also an unavoidable result of the source of the oxocarbon having a variable pressure (e.g., an industrial waste source) and therefore must be tolerated when processing the oxocarbons.

In specific embodiments of the invention, an electrolysis reactor includes an anode area and a cathode area with a porous separator separating the anode area and the cathode

area. The porous separator can have pores with cross sections having an average size less than one millimeter down to hundreds of nanometers. The porous separator can include a porous network formed by a set of such pores that extend through the separator from one side of the separator to another side of the separator. The porous network extends through the separator in that there are paths from the one side of the separator to the other side of the separator through the porous network. In specific embodiments of the invention, this porous network can be filled with a liquid electrolyte after the separator is installed in the electrolyzer. Using the approaches disclosed herein, an electrolysis reactor can thereby provide for facile migration of ionic species between the anode and cathode to improve the performance of the electrolyzer. In specific embodiments of the invention, an electrolysis reactor can utilize an electroneutral porous separator. The electroneutral separator can be formed by electrically insulative material while being ionically conductive via the migration of ions through the porous network. A conductive electrolyte of the electrolysis reactor can fill the pores of the separator to provide a path for ions to migrate through the separator.

In specific embodiments of the invention, an electrolysis reactor includes an anode area and a cathode area separated by a porous separator where one of the two areas is an aqueous area and the other of the two areas is a gaseous area. The anode area could be an aqueous anode area and the cathode area could be a gaseous cathode area or vice versa. In these embodiments, a pump or other means can be used to produce a pressure difference across the electrolysis reactor from the anode area to the cathode area. A conductive electrolyte, or any other fluid, located in the aqueous area can be pressed away from the gaseous area by the pressure difference such that the fluid is kept in the porous separator, but does not extend into the gaseous area. Adjusting the pressure difference can adjust a degree of interactivity with the conductive electrolyte and a catalyst layer of the anode area or cathode area.

In specific embodiments of the invention, the separators disclosed herein can be coated with a coating to improve the performance of the oxocarbon electrolysis reactor in which the separator is utilized. The coating can be selected such that it increases the hydrophilicity of the separator such as by increasing the hydrophilicity of the surfaces of the pores in a porous separator. The coating can be selected such that it can withstand contact with the electrolyte of an oxocarbon electrolysis reactor, can withstand oxidation, and can withstand the general conditions of a separator in an oxocarbon electrolysis reactor such that the coating stays on the separator and the performance of the separator does not degrade during usage of the separator in an oxocarbon electrolysis reactor. The coatings can be selected to be nonionic at neutral pH, water insoluble, water immiscible, soluble in small alcohols (e.g., ethanol and isopropanol), non-volatile, stable in metal hydroxide solutions, and contain at least one polar function group. The coating can also be selected to have a similar chemical structure as the separator to assure the coating meshes well with the separator. In specific embodiments, both the material of which the separator is formed, and the coating, can be selected in combination to assure good adherence of the coating to the separator and improved performance of the oxocarbon electrolysis reactor.

In specific embodiments of the inventions disclosed herein, an oxocarbon electrolysis reactor is provided. The oxocarbon electrolysis reactor comprises an aqueous anode area with an oxidation substrate, a gaseous cathode area with an oxocarbon species as a reduction substrate, and an

electroneutral separator separating the aqueous anode area and the gaseous cathode area while allowing ionic migration between the aqueous anode area and gaseous cathode area. The electroneutral separator is a polymer having a coating. 5 The coating is formed of an aliphatic molecule. The coating increases a hydrophilicity of the electroneutral separator.

In specific embodiments of the inventions disclosed herein, an oxocarbon electrolysis reactor is provided. The oxocarbon electrolysis reactor comprises an aqueous anode area with an oxidation substrate, a gaseous cathode area with an oxocarbon species as a reduction substrate, and an electroneutral separator separating the aqueous anode area and the gaseous cathode area while allowing ionic migration between the aqueous anode area and gaseous cathode area. 10 The electroneutral separator is a polymer having a coating. The polymer is composed of aliphatic carbons. The coating is an aliphatic carbon chain with a hydrophilic functional group.

In specific embodiments of the inventions disclosed herein, a method of operating an oxocarbon electrolysis reactor is provided. The method comprises reducing an oxocarbon species in a gaseous cathode area, oxidizing an oxidation substrate in an aqueous anode area, separating the 15 gaseous cathode area from the aqueous anode area using an electroneutral separator, and allowing ionic migration between the aqueous anode area and gaseous cathode area across the electroneutral separator. The electroneutral separator is a polymer having a coating. The polymer comprises 20 a linear aliphatic carbon chain. The coating is a linear aliphatic carbon chain with a hydrophilic functional group.

#### BRIEF DESCRIPTION OF THE DRAWINGS

35 The accompanying drawings illustrate various embodiments of systems, methods, and other aspects of the disclosure. A person with ordinary skills in the art will appreciate that the illustrated element boundaries (e.g., boxes, groups of boxes, or other shapes) in the figures represent one 40 example of the boundaries. It may be that in some examples one element may be designed as multiple elements or that multiple elements may be designed as one element. In some examples, an element shown as an internal component of one element may be implemented as an external component in another and vice versa. Furthermore, elements may not be drawn to scale. Non-limiting and non-exhaustive descriptions are described with reference to the following drawings. The components in the figures are not necessarily to scale, emphasis instead being placed upon illustrating principles.

45 FIG. 1 illustrates an oxocarbon electrolysis reactor that can be utilized in accordance with specific embodiments of the inventions disclosed herein.

50 FIG. 2 includes two block diagrams of electrolysis reactors in accordance with the related art.

55 FIG. 3 includes a block diagram of an electrolysis reactor with a porous electroneutral separator and two illustrations of a separator in accordance with specific embodiments of the inventions disclosed herein.

60 FIG. 4 illustrates a network of pores in a diaphragm and a pore having a coating in accordance with specific embodiments of the inventions disclosed herein.

65 FIG. 5 illustrates chemical reactions of candidate coating materials in accordance with specific embodiments of the inventions disclosed herein.

66 FIG. 6 illustrates chemical structures of candidate coating materials in accordance with specific embodiments of the inventions disclosed herein.

FIG. 7 illustrates the cell potential and Faradic efficiency for ethylene and dihydrogen conversion of oxocarbon reactors having polyethylene separators that are coated with four different percentage by weight wt % values of a solution having a coating of octadecan-1-ol in accordance with specific embodiments of the inventions disclosed herein.

FIG. 8 illustrates the cell potential and Faradic efficiency for ethylene and dihydrogen conversion of an oxocarbon reactor having a polyethylene separator that is coated with a 0.01 wt % coating solution of PEVA in accordance with specific embodiments of the inventions disclosed herein.

FIG. 9 illustrates the cell potential and Faradic efficiency for ethylene and dihydrogen conversion of an oxocarbon reactor having a polyethylene separator that is coated with a 1 wt % coating solution of PEVA that was subsequently reacted with glutaraldehyde in accordance with specific embodiments of the inventions disclosed herein.

FIG. 10 illustrates the cell potential and Faradic efficiency for ethylene and dihydrogen conversion of oxocarbon reactors where one reactor has a Piperion AEM, and two reactors have polyethylene separators that are coated with two different coatings in accordance with specific embodiments of the inventions disclosed herein.

FIG. 11 illustrates the cell potential and Faradic efficiency for ethylene and dihydrogen conversion of oxocarbon reactors having a 4M concentration of electrolyte where one reactor has a Piperion AEM and the other has a polyethylene separator coated in trihexylamine in accordance with specific embodiments of the inventions disclosed herein.

FIG. 12 includes a block diagram of a carbon dioxide electrolysis reactor in accordance with specific embodiments of the inventions disclosed herein.

FIG. 13 includes a block diagram of a carbon monoxide electrolysis reactor in accordance with specific embodiments of the inventions disclosed herein.

FIG. 14 includes a block diagram of an electrolysis reactor where an electrolyte is applied directly to a separator in accordance with specific embodiments of the inventions disclosed herein.

FIG. 15 includes a flow chart for a set of methods for operating an electrolysis reactor in accordance with specific embodiments of the inventions disclosed herein.

#### DETAILED DESCRIPTION

Reference will now be made in detail to implementations and embodiments of various aspects and variations of systems and methods described herein. Although several exemplary variations of the systems and methods are described herein, other variations of the systems and methods may include aspects of the systems and methods described herein combined in any suitable manner having combinations of all or some of the aspects described.

Methods and systems related to novel separators and oxocarbon electrolysis reactors utilizing such novel separators in accordance with the summary above are disclosed in detail herein. The methods and systems disclosed in this section are nonlimiting embodiments of the invention, are provided for explanatory purposes only, and should not be used to constrict the full scope of the invention. It is to be understood that the disclosed embodiments may or may not overlap with each other. Thus, part of one embodiment, or specific embodiments thereof, may or may not fall within the ambit of another, or specific embodiments thereof, and vice versa. Different embodiments from different aspects may be combined or practiced separately. Many different combinations and sub-combinations of the representative embodi-

ments shown within the broad framework of this invention, that may be apparent to those skilled in the art but not explicitly shown or described, should not be construed as precluded.

5 The electrolyzers used in accordance with the approaches disclosed herein can have various architectures. The electrolyzer can include an anode area and a cathode area. An oxocarbon can be provided to the cathode area of the reactor as a reduction substrate. Useful chemicals can be produced 10 in the cathode area, in the anode area, or in a separating area located between the cathode area and the anode area of the electrolyzer. The rate at which the reaction occurs can be dependent upon the degree of ionic migration across one or more separators between the cathode area and the anode area. 15 The electrolyzer can be a single planar electrolyzer. The electrolyzer can be a stack of cells. The cells in the stack can utilize bipolar plates. The bipolar plates can be charged to initiate reactions within the reactor. The electrolyzer can also be a filter press electrolyzer or a tubular electrolyzer. 20 The electrolyzers used in accordance with this disclosure can comprise one or more electrocatalytic cells positioned on top or next to one another to increase the surface available for the reaction. They can be stacked on top of one another, and such stacks can also be parallelized. These cells 25 may be connected in series or in parallel. Many different cell and stack configurations can be used for the electrolyzers in accordance with this disclosure. FIG. 1 illustrates an oxocarbon electrolysis reactor 100 that can be utilized in accordance with specific embodiments of the inventions disclosed herein for explanatory purposes. The methods and systems disclosed herein are broadly applicable to oxocarbon electrolyzers generally and oxocarbon electrolysis reactor 100 is provided as a nonlimiting example of one such electrolyzer.

30 FIG. 1 includes an illustration of an oxocarbon electrolysis reactor 100 in the form of a stack in accordance with specific embodiments of the inventions disclosed herein. The oxocarbon electrolysis reactor 100 includes end plates such as end plate 102, monopolar plates such as monopolar plate 104, rigid bars such as rigid bar 106, a separator and electrode assembly such as electrode assembly 108, a flow field such as flow field 110, and bipolar plates such as bipolar plate 112. Additionally, the oxocarbon electrolysis reactor 100 includes an inlet 114 and an outlet 116 for an anodic stream, as well as an inlet 118 for a cathodic stream and an 35 outlet 120 for the cathodic stream. An oxocarbon can be provided at the inlet 118 in the cathodic stream. The oxocarbon can be humidified. A useful chemical can be provided at outlet 116 in the anodic stream. The polar plates, such as monopolar plate 104 and bipolar plate 112 can be part of the 40 cells in the stack. The stack can also comprise gasketing, scaling of any shape, insulating layers and other materials that have not been represented in the FIG. 1 for clarity.

45 In an electrolysis stack, subsequent cells can be physically separated by bipolar plates (BPPs), such as bipolar plate 112 in FIG. 1, that can ensure mechanical support for each of the electrolysis cells on each side of the BPP. BPP can also ensure electrical series connection between subsequent electrolysis cells and introduce/remove the reactants/products 50 respectively. At the end of the stack, only one side of the plate can be in contact with the terminal cell; it is then called a monopolar plate, such as monopolar plate 104 in FIG. 1. At the extremities of the stack, current collectors can allow connection to an external power supply, which can also be used, among other elements, for electrical monitoring of the 55 stack. The stack can be assembled within a stack casing allowing its mechanical support and compression, as well as provisioning and transporting the reactant and product

streams to and from the stack. The stack casing can comprise end plates that ensure electrical isolation of the stack and provide the inlet and outlets for the reactant and product streams. Alternatively, insulator plates can be placed between the end plates such as end plate 102 and the monopolar plate such as monopolar plate 104 to ensure electrical insulation of the stack versus the stack casing depending on the material of the end plate.

The carbon monoxide electrolyzers can take as an input, a cathodic input stream (e.g., stream enriched in carbon monoxide) and an anode input stream. In such case, the reduction substrate is carbon monoxide. The cathodic input stream can be provided to an inlet such as inlet 118. The anodic input stream can be provided to an inlet such as inlet 114. The cathodic stream and anodic stream can flow through the stack from the inlets to the outlets and be distributed through the flow channels, such as those in flow field 110 of each cell to each cathodic and anodic area separately. The anodic stream and cathodic stream would flow through separate channels on either side of the cell. Alternatively, at least one of the cathodic and anodic streams may be provided to each cell individually instead of through a connection crossing all the plates. In this case, each cell has a dedicated fluid inlet and outlet for this cathodic and/or anodic stream. The nature of the anodic stream can be determined by the nature of the targeted oxidation reaction (such as, but not limited to, water oxidation, dihydrogen oxidation, chloride oxidation, halide oxidation, hydrocarbon oxidation, and waste organic oxidation). For example, the generating of chemicals using carbon monoxide and the electrolyzer could involve supplying the volume of carbon monoxide to a cathode area of the electrolyzer as a cathodic input fluid and supplying a volume of water to an anode area of the electrolyzer as an anodic input fluid. When electrically powered, the carbon monoxide electrolyzer carries out the concomitant reduction of carbon monoxide and oxidation of the chosen oxidation substrate to produce added-value chemicals such as hydrocarbons, organic acids and/or alcohols and/or N-containing organic products in the anodic stream.

In specific embodiments of the inventions disclosed herein, the electrolyzer can be operated at elevated temperature and pressure to promote the stability and performance of the electrolyzer by improving oxocarbon mass transport and product efflux. Elevated temperature can serve to evaporate liquid products present in the cathode catalyst layer, while elevated pressure can mitigate the intrusion and retention of liquids in the cathode catalyst layer. In specific embodiments, the electrolyzer can be operated under elevated pressure at both the anode and cathode compartments, or only in one compartment. In embodiments in which the electrolyzer is a mixed liquid and gas phase electrolyzer, elevating pressure in a single compartment could be used to precisely manage liquid and gas crossover in the electrolyzer. In particular, if the separator were a porous separator and the electrolyzer were a mixed liquid and gas phase electrolyzer, a pressure differential could be formed in the electrolyzer to keep the electrolyte pressed away from the gas phase compartment of the electrolyzer.

In specific embodiments of the invention, the electrolyzer can include one or more separators separating the anode area and the cathode area such as separator 130 in the separator and electrode assembly 108. As illustrated, separators such as separator 130 can provide sufficient mechanical stability such that they may serve to support an electrode on both the anode side and cathode side of the electrolyzer. The separation can be conducted to isolate specific generated chemi-

cals from others (e.g., a useful chemical produced at the anode from a byproduct produced at the cathode). The separation can be conducted to provide mechanical stability to the electrolyzer cell in which the separator is used. The separation can be conducted to maintain the different chemistries required for the reduction reaction to occur in the cathode area and the oxidation reaction to occur in the anode area. The separation can also be conducted to prevent short-circuiting contact between anode and cathode layers and prevents crossover of gaseous products generated at the anode and cathode to the opposite electrode. The one or more separators can separate the anode area and the cathode area by being located between the anode area and the cathode area. The electrolyzer may also include a separating area between the anode area and the cathode area configured to separate a volume of generated chemicals from the electrolyzer. The separating area can be isolated from the cathode and/or anode using one or more separators. For example, a first separator could be located at an interface between the separating area and the anode area while another separator could be located at an interface between the separating area and the cathode area. Regardless, as the terms are used herein, a separator "separates the anode area and the cathode area" if it is located at least partly between the cathode area and the anode area. As such, the two separators in the prior example serve to separate the anode area and the cathode area regardless of the fact that each one is not physically in contact with either the anode area or the cathode area because they are both still located at least partly between the anode area and the cathode area.

As mentioned in the summary above, the separator can be an electroneutral separator. The electroneutral separator can be ionically conductive while still providing high mechanical stability. For example, the electroneutral separator can be strong enough to withstand a pressure differential of 300 mbar without being deformed. The separator can be a porous separator. The separator can be an electroneutral porous separator. The separator can have a conductive electrolyte which fills the pores in the porous separator. The porous electroneutral separator can provide ionic conductivity by having a network of pores that include paths which extend from one side of the separator to the other side of the separator through the network of pores. This ionic conductivity can be provided by a conductive electrolyte which fills the network of pores. Further details regarding the separators and their properties are provided in detail below.

As mentioned above, the oxocarbon electrolyzers can be used to produce useful chemicals. An oxocarbon electrolyzer in accordance with specific embodiments disclosed herein can include a cathode area where carbon oxide (e.g., carbon dioxide and/or carbon monoxide) reduction takes place, according to equation 1 and 2 below, and an anode area where an oxidation reaction takes place on an oxidizing catalyst. The oxidation substrate can be water, dihydrogen gas, halides, organic waste, or any other oxidation substrate. For example, the oxidation can involve water oxidation or dihydrogen oxidation according to equations 3 and 4 below respectively.



The reactions below can be conducted in accordance with the electrolyzers described herein. In the diagrams provided herein, only single cells are represented for clarity, but these could be assembled in a plurality of cells, such as in an electrolyzer stack. In the diagrams, a carbon oxide electrolyzer comprises a cathode comprising a gas-diffusion layer and a cathode catalyst, and the anode comprises an anode catalyst deposited on a transport layer of any shape (such as but not limited to a foam, a mesh, a deposit onto a conductive porous transport layer (PTL), etc.). In this case, the carbon oxide reduction products include one or more of the following: carbon monoxide (CO), syngas (CO+H<sub>2</sub>), ethylene (C<sub>2</sub>H<sub>4</sub>), ethanol (C<sub>2</sub>H<sub>5</sub>OH), acetic acid (CH<sub>3</sub>COOH), propylene (C<sub>3</sub>H<sub>6</sub>), propanol (C<sub>3</sub>H<sub>8</sub>O), oxalic acid (COOH-COOH), acrylic acid (C<sub>2</sub>H<sub>3</sub>COOH), and glyoxylic acid (COH-COOH) produced according to the following reduction reactions. In neutral/alkaline conditions for CO<sub>2</sub> reduction:



In neutral/alkaline conditions for CO reduction:



The electrode may also generate syngas, a mixture of H<sub>2</sub> and CO through a concomitant production of H<sub>2</sub> through reaction 18 with reaction 5.



In tandem, the anode carries out an oxidation reaction at the anode from the group consisting of reactions such as but not limited to:



These reactions are assisted catalytically by the presence of metal cations, such as, but not exclusively Li<sup>+</sup>, Na<sup>+</sup>, K<sup>+</sup>, Rb<sup>+</sup>, Cs<sup>+</sup>, and Fr<sup>+</sup>. The presence of these cations can be enabled through the liquid phase of the reactor, which is typically introduced at the anode area, but may be introduced at a central separator or cathode area of the reactor. These cations can reach the cathode catalyst layer via diffusion across an electroneutral separator between the anode area and the cathode area. At the same time, an electroneutral separator can allow the ions from the reduction and/or oxidation reactions occurring at the electrolyzer's catalytic electrodes to be transferred across the electrolyzer (e.g., ions such as H<sup>+</sup>, CO<sub>3</sub><sup>2-</sup>, OH<sup>-</sup>, or HCO<sup>3-</sup> can migrate across the separator).

In specific embodiments of the invention, a separator in accordance with this disclosure allows for indiscriminate movement of ions across the separator through a network of pores. The network of pores may include a network of submillimeter interconnected pores forming paths through the separator. The network of pores may be formed by an insulating material that provides the structure of the separator. The insulating material may form an insulating network containing for example, carbon, oxygen, fluorine, hydrogen, silicon, and nitrogen bonds. The pores in the network of pores accumulate liquid electrolyte that allows the flow of both anions and cations to the anode area and cathode area respectively. Unlike in ion exchange membranes, this leads to a separator that does not hinder the flow of a particular ionic species. Such an alternative is illustrated by electrolyzer 200 in FIG. 2 having an anion exchange membrane 201 separating a cathode area 202 from an anode area 203 and electrolyzer 210 having a cation exchange membrane 211 separating a cathode area 212 from an anode area 213. This can be contrasted with the electrolyzer 300 in FIG. 3 where an electroneutral separator 301 allows for the facile migration of both anions and cations between cathode area 302 and anode area 303. In the illustrated electrolyzer diagrams dotted arrows represent electrochemical conversions while solid arrows represent ionic diffusion. FIG. 3 also includes a separator surface view 310 which shows a set of pores including pore 311 and a cross section of the separator 320 showing a porous network 321 formed by the set of pores and extending through the separator from an anode side 322 to a cathode side 323. The network includes a set of paths such as path 324 that extend from the anode side to the cathode side.

The pores in the separator can take on various forms in different embodiments of the invention. In specific embodiments of the invention, a porous separator works by providing optimally sized pores in which electrolyte may be trapped to allow ion flux in both directions across the electrolyzer. In specific embodiments, this functionality enables the diffusion of alkali metal cations to accumulate at the cathode catalyst of the electrolyzer which are used by the cathode catalyst to undertake oxocarbon reduction. The pores also allow the flow of anions that are generated from the reduction reaction at the cathode to flow to the anode. The pores in the separator can be regularly spaced or irregularly spaced depending upon how they are formed. The pores can be various sizes as set by the desired mechanical stability and ionic conductivity of the separator. The pores in the set of pores can be submillimeter scale and can

## 11

have an average size less than one millimeter. The pores can be micron scale pores. The pores can be as small as 200 nanometers or smaller. The pores can be exposed on the surface of the separator such that when the separator is brought into contact with a liquid, such as a conductive electrolyte in the anode area or cathode area of the electrolyzer, the liquid fills the pores and thereby extends through the porous separator via the porous network. In embodiments in which the pores form a porous network, the network can be filled with a conductive electrolyte.

In specific embodiments of the invention, a porous sheet of natural, synthetic, or semisynthetic polymeric material is used as the separator. In specific embodiments, the separators will be electroneutral separators that do not include any charged particles implanted into the material (e.g., polymer(s) used to form the separator). The separator can be formed of various polymeric materials such as, but not exclusively, by one or more polymers selected from the group consisting of polytetrafluoroethylenes, polyethylenes, polypropylenes, polystyrenes, polysiloxanes, polyether sulfone, polacrylonitrile, polyacrylates, polyimides, polycarbonates or cellulose acetates, or any mixture thereof. The separator can be formed of polymer composed of one or more monomers selected from a group consisting of: tetrafluoroethylenes, ethylenes, propylenes, polystyrenes, polysiloxanes, polacrylonitrile, polyacrylates, sulfones, polyimides, polycarbonates, and cellulose acetates. The separator may also include porous ceramic materials and/or a mixture of polymeric and ceramic materials. These polymers can be fabricated into thin films containing pores on the submillimeter scale. The polymers may be used alone or may be copolymerized with other materials to attain the desired structural and mechanical properties for a given electrolyzer. The separator can be a polymer formed by chain growth polymerization of one or more monomers selected from a group consisting of: vinyls, olefins, styrenes, acrylates, methacrylates, acrylamides, methacrylamides, epoxides, lactones, lactams, siloxanes, sulfones, and carbonates. The separator can be a polymer formed by step growth polymerization of one or more chemicals selected from a group consisting of multifunctional alcohols, amines, thiols with one or more multifunctional carboxylic acids, acid halides, alkyl halide, esters, isocyanates, aldehydes, ketones, or anhydrides.

In specific embodiments of the invention, the polymeric separator may be functionalized with a coating to render the separator more hydrophobic or hydrophilic, through functionalization with organic or inorganic additives. The coating can increase the hydrophilicity or hydrophobicity of the separator. The coating can be an uncharged polymer, a nonionic surfactant, a wax, an alcohol, an amine, a thiol, an ether, an ester, an amide, a nitrile, an imide, a phosphine, or a mixture thereof. The separators may also be adorned with catalyst particles or other transition metal species both inside and on the outer faces of the separator to facilitate charge and ion transfer reactions and the electrolyzer's catalytic interfaces. Coating of the separator may be achieved through a technique such as doctor blading, electrospinning, spin coating, evaporation, drop casting, spray-coating, or by immersing the separator into a liquid form of solution of the species to be coated. In some cases, the coating may be necessary for the separator to function in the carbon oxide electrolyzer.

In specific embodiments of the invention, the coating can be selected such that it increases the hydrophilicity of the separator such as by increasing the hydrophilicity of the surfaces of the pores in a porous separator. The coating can be selected such that it can withstand contact with the

## 12

electrolyte of an oxocarbon electrolysis reactor, can withstand oxidation, and can withstand the general conditions of a separator in an oxocarbon electrolysis reactor such that the coating stays on the separator and the performance of the separator does not degrade during usage of the separator in an oxocarbon electrolysis reactor. The coatings can be selected to be nonionic at neutral pH, water insoluble, water immiscible, insoluble or sparingly soluble in small alcohols (e.g., ethanol and isopropanol), non-volatile, stable in metal hydroxide solutions, and contain at least one polar function group. Coating materials that satisfy the above requirements and have been found to perform well in an oxocarbon electrolyzer include aliphatic molecules selected from the group consisting of aliphatic alcohols, aliphatic amines, aliphatic ethers, aliphatic acetals, and aliphatic ketals. Linear, branched, and cyclic aliphatic alcohols, aliphatic amines, and aliphatic ethers have been found to be effective. Primary, secondary, and tertiary alcohols and amines have been found to be effective. Aliphatic thiols were also tested and functioned but did not perform as well. Aliphatic nitriles are also expected to function well.

Polymeric molecules have also been found to be effective additives to use as coatings for electroneutral porous separators. These polymeric additives can be selected to be nonionic at neutral pH, water insoluble, water immiscible, insoluble or sparingly soluble in small alcohols (e.g., ethanol and isopropanol), non-volatile, stable in metal hydroxide solutions, and contain at least one polar function group. Linear, branched, and cyclic aliphatic polymeric chains with pendant hydrophilic groups have been found to be effective. The ratio of aliphatic polymeric chain to pendant hydrophilic groups should be such that the molar ratio of ethylene is high enough to render the additive suitably hydrophobic that is insoluble in water. Polymeric additives that have been found most effective are based on polyethylene as the aliphatic chain and vinyl alcohol groups as the pendant hydrophilic group.

Separator coatings composed of polymeric molecules may also be modified further by reacting the pendant hydrophilic groups to improve the coatings performance. This modification can be used to increase or decrease the hydrophilicity of the coating to ensure the polymeric additive is nonionic at neutral pH, water insoluble, water immiscible, insoluble or sparingly soluble in small alcohols (e.g., ethanol and isopropanol), non-volatile, stable in metal hydroxide solutions, and contain at least one polar function group. Modification reactions that have been found to be useful are reactions of pendant alcohols with aldehydes and ketals to form acetals and ketals, respectively. These molecules used to modify the polymeric coating molecule may contain one or more aldehydes or ketones. Multiple aldehydes and ketones on a single molecule can be used to cause cross-linking of the polymeric coating molecule.

In specific embodiments of the invention, the coating can be selected to be one of the specific chemicals listed in the following table. The coatings will be referred to using the chemical formulas presented in the third column. Each of these chemicals includes an aliphatic functional group that is either an aliphatic alcohol, ether, amine, acetal, or ketal. All the chemicals listed have been proven to be effective at increasing the hydrophilicity of a separator, to be stable during oxocarbon electrolysis, and to meet the requirements listed in the prior paragraphs.

| Name                                                            | Functional Group                                  | Formula | Chemical Structure |
|-----------------------------------------------------------------|---------------------------------------------------|---------|--------------------|
| Octadecan-1-ol                                                  | Aliphatic primary alcohol                         | OdOH    |                    |
| 2-Methylnonadecan-2-ol                                          | Aliphatic tertiary alcohol                        | MeNdOH  |                    |
| 1-Methoxyhexane                                                 | Aliphatic ether                                   | MeOHx   |                    |
| Trihexylamine                                                   | Aliphatic tertiary amine                          | THxA    |                    |
| Poly(ethylene-co-vinyl alcohol)                                 | Aliphatic secondary alcohol                       | PEVA    |                    |
| Poly(ethylene-co-vinyl alcohol) crosslinked with glutaraldehyde | Aliphatic secondary alcohol and aliphatic acetals | PEVA-GA |                    |

In specific embodiments, the material for the separator can be selected to have certain characteristics to improve the performance of the oxocarbon electrolyzer in which it is used. The separator can be nonionic, be water insoluble, exhibit little to no swelling in water, be insoluble in alcohols (e.g., ethanol and isopropanol), be stable in metal hydroxide solutions, be oxidatively stable, be capable of being cast into a porous membrane, and be mechanically strong. Separators that satisfy the above requirements and that were shown to perform well in oxocarbon electrolyzers include polyethylene. Separators that functioned but did not perform as well as polyethylene include polytetrafluoroethylene, and polypropylene. Poly(styrene), poly(styrene-*b*-(ethylene-*co*-butylene)-*b*-styrene), poly(styrene-*co*-butadiene), poly(ethylene-*co*-propylene), polysiloxanes are also expected to form separators that function well in an oxocarbon electrolyzer in accordance with the principles disclosed herein.

Oxocarbon electrolyzers and water electrolyzers can use charged membranes such as an anionic exchange membrane (AEM) or a diaphragm to separate the electrodes and facilitate the transport of ions across from anode to cathode or vice versa. Schematic differences between AEMs and diaphragms are shown in FIG. 4. As illustrated in FIG. 4, a network of pores in a diaphragm 400 and a set of channels

in an AEM 410 both allow for the migration of anions (i.e., hydroxide anions in the illustrated case). However, a diaphragm also allows for the migration of cation (i.e., potassium cations in the illustrated case). A conceptual diagram 450 of a pore including a separator material 452 in the form of polyethylene with a coating 451 in the form of OdOH is 45 also provided in the diagram. While conceptual diagram 450 shows the pore extending all the way from the anode to the cathode, it is more realistic for a network of interconnected pores would reach from the anode to the cathode. Diaphragms are porous inert materials that fill with electrolyte 50 (e.g., a solution with potassium cations and hydroxide anions) and allow the cations and anions to move across the cell to allow current to flow. Essentially, diaphragms are there to provide a solid support to contain liquid electrolyte. Diaphragms can be combined with other materials to 55 augment the properties. AEMs also have a solid phase but they contain positive charges that are chemically bound to the solid phase surface (e.g., the cations bound to the solid phase of the separator in AEM 410). AEMs will absorb water 60 (because the positive charges are hydrophilic) but the polymer will not dissolve (because there is a solid hydrophobic phase). These positive surface charges allow a site for anions

(e.g., hydroxide as shown in the diagram) to move across the surface and through the membrane to the anode from the cathode.

In specific embodiments disclosed herein, a combination of the AEM approach illustrated by AEM **410** and the diaphragm approach of diaphragm **400** utilizes a solid separator material coated with a coating such as in the case of diagram **450**. In the illustrated approach, a diaphragm type separator of polyethylene is exposed to a coating material to modify the pore surface with said coating to render the pore surface water wet. FIG. 4 depicts a separator material **452** of polyethylene with a coating **451** of OdOH. The OdOH illustrates a principle of the chemicals listed for coatings provided above in that it contains one hydrophilic functional group (e.g., an alcohol, an ether, or an amine) that is hydrophilic. Ideally these water wet pores allow the polyethylene to fill with electrolyte during electrolysis and allow ions to flow freely from one electrode to the other during electrolysis. As such, the coating plays the role of the cations bound to the solid phase separator in AEM **410**, without the need for expensive procedures to incorporate charge onto the membrane.

In specific embodiments of the invention, the coating should be adsorbed strongly to the separator material and should not be removed by electrolysis. In specific embodiments, the coating can also be selected to have a similar chemical structure as the separator to assure the coating meshes well with the separator. In specific embodiments, both the material of which the separator is formed, and the coating, can be selected in combination to assure good adherence of the coating to the separator and improved performance of the oxocarbon electrolysis reactor. For example, polyethylene and the additives listed in the table above work well because the chemistry of the polyethylene and the additives are very similar. Polyethylene is entirely a linear aliphatic carbon chain, and the coating materials are predominately linear aliphatic carbon chains. Therefore, there is strong adsorption between the coating materials and the polyethylene. Furthermore, it is likely that the hydrophilic functional group of the coating will orientate away from the hydrophobic surface and present a hydrophilic surface inside the pore. This is beneficial in that, as described above with reference to FIG. 4, the pores are thereby water wettable and capable of filling with electrolyte necessary for electrolysis.

As stated previously, the coatings can be selected to prevent chemical degradation when utilized in an oxocarbon electrolyzer. For example, the coating can be selected to prevent degradation after being attacked by hydroxide present in the electrolysis. As such, certain chemical functionalities such as esters and amides should be avoided. FIG. 5 illustrates the base hydrolysis of an aliphatic ester to potassium carboxylic acid salt and a primary alcohol **500**. Although the initial aliphatic ester may perform well as a coating the gradual hydrolysis over operation will change the performance of the separator. Furthermore, the hydrolysis products are more water soluble and will gradually be removed from the surface of the separator. Removal of these species, and other coatings, from the surface reduces the hydrophilicity of the separator. As another example, the coating should be selected such that it is oxidatively stable. FIG. 5 also illustrates the oxidation of a sulfide through multiple oxidation steps which eventually transform the sulfide into a sulfone via a sulfoxide **510**. Gradual oxidation of the coating during operation is not suitable as this will change the separators performance over time and may increase the coating's water solubility, eventually leading to

the coating washing off. As another example, the coating should be selected such that it remains nonionic. FIG. 5 also illustrates how a thiol can be deprotonated to a thiolate when exposed to a base such as potassium hydroxide **520**. The resulting thiolate would not only be more water soluble and dispersible it would also be a strong nucleophile and may react with other molecules present, such as carbon monoxide.

FIG. 6 illustrates chemical structures of candidate coating materials in accordance with specific embodiments of the inventions disclosed herein. As mentioned previously, the coating and separator chemistries can be selected to be similar to enhance the potential for strong adsorption of the coating chemical to the separator. In the case of polytetrafluoroethylene a coating that was itself fluorinated and that had a polar group to provide hydrophilicity would perform well. The chemical structure of a separator of polytetrafluoroethylene **600** and a coating of fluorinated alcohol **610** are provided in FIG. 6 as an illustration of such a potential combination. Generally, separator materials with branched structures, such as polypropylene (structure shown as **620** in FIG. 6) as opposed to linear structures, such as polyethylene (structure shown as **640** in FIG. 6) may be more difficult to pair with a well adsorbing coating because the coating molecules are not able to stack well onto the separator.

Certain combinations of separators and coatings disclosed herein have some advantages over other AEMs formed by materials such as Piperion for oxocarbon electrolysis for several reasons. Firstly, cationic groups on Piperion will gradually be degraded by hydroxide ions, degradation is accelerated at increased concentrations of hydroxide ions or temperature. Piperion can dissolve/disperse in ethanol which is a co-product during the electrolysis of carbon monoxide. Electrolysis of carbon monoxide can produce ethanol and 1-propanol as co-products, and these alcohols in the presence of potassium hydroxide will form small amount of alkoxides in solution that are very basic and can degrade the cationic group of Piperion. Furthermore, Piperion, and similar cationically charged membranes, are relatively expensive compared to some of the electroneutral separators disclosed herein. Finally, Piperion is not as mechanically strong as separators and has been shown to suffer mechanical failure during operation, causing electrical short circuits or allowing gas to crossover via the broken membrane.

FIG. 7 illustrates the cell potential and Faradic efficiency for ethylene and dihydrogen conversion of oxocarbon reactors having polyethylene separators that are coated with four different wt % values of a coating of OdOH in accordance with specific embodiments of the inventions disclosed herein. The current density applied to the reactors was 200 mA per centimeter squared of active area on the scale of five centimeters squared. The anolyte in both reactors was 1 M potassium hydroxide. The x-axis of both plots is time in hours. Line **700** shows the potential voltage across the cell for a 2.5 wt % coating of OdOH, line **710** shows the potential voltage across the cell for a 0.5 wt % coating of OdOH, line **711** shows the potential voltage across the cell for a 0.04 wt % coating of OdOH, and line **712** shows the potential voltage across the cell for a 5 wt % coating of OdOH.

The carbon monoxide reduction performance of the separators varies with the wt %. Line **721** shows the ethylene Faradaic efficiency of the 0.04 wt % separator reactor. Line **722** shows the hydrogen Faradaic efficiency of the 0.04 wt % separator reactor. Line **723** shows the ethylene Faradaic efficiency of the 0.5 wt % separator reactor. Line **724** shows the hydrogen Faradaic efficiency of the 0.5 wt % separator reactor. Line **725** shows the ethylene Faradaic efficiency of

the 2.5 wt % separator reactor. Line 726 shows the hydrogen Faradaic efficiency of the 2.5 wt % separator reactor. Line 727 shows the ethylene Faradaic efficiency of the 5 wt % separator reactor. Line 728 shows the hydrogen Faradaic efficiency of the 5 wt % separator reactor.

FIG. 8 illustrates the cell potential and Faradic efficiency for ethylene and dihydrogen conversion of an oxocarbon reactor having a polyethylene separator that is coated with a coating solution of 0.01 wt % PEVA in accordance with specific embodiments of the inventions disclosed herein. The current density applied to the reactor was 200 mA per centimeter squared of active area on the scale of five centimeters squared. The anolyte in the reactor was 1 M potassium hydroxide. The x-axis of both plots is time in hours. Line 800 shows the potential voltage across the cell for a 0.01 wt % coating of PEVA. Line 801 shows the ethylene Faradaic efficiency of the reactor. Line 802 shows the hydrogen Faradaic efficiency of the reactor.

FIG. 9 illustrates the cell potential and Faradic efficiency for ethylene and dihydrogen conversion of an oxocarbon reactor having a polyethylene separators that is coated with a 1 wt % coating solution of PEVA that was subsequently reacted with glutaraldehyde in accordance with specific embodiments of the inventions disclosed herein. The current density applied to the reactor was 200 mA per centimeter squared of active area on the scale of five centimeters squared. The anolyte in the reactor was 1 M potassium hydroxide. The x-axis of both plots is time in hours. Line 901 shows the potential voltage across the cell for a 1 wt % coating of PEVA subsequently reacted with glutaraldehyde. Line 902 shows the ethylene Faradaic efficiency of the reactor. Line 903 shows the hydrogen Faradaic efficiency of the reactor.

FIG. 10 illustrates the cell potential and Faradic efficiency for ethylene and dihydrogen conversion of oxocarbon reactors. A first reactor has a Piperion AEM. A second reactor has a polyethylene separator coated with a 0.5 wt % OdOH solution. A third reactor has a polyethylene separator coated with a 0.5 wt % THxA solution. The current density applied to the reactors was 200 mA per centimeter squared of active area on the scale of five centimeters squared. The anolyte in both reactors was 2 M potassium hydroxide. The x-axis of both plots is time in hours. Line 1000 shows the potential voltage across the cell for the Piperion separator. Line 1010 shows the potential voltage across the cell for a 0.5 wt % coating of OdOH. Line 1020 shows the potential voltage across the cell for a 0.5 wt % coating of THxA. Line 1031 shows the ethylene Faradaic efficiency of the Piperion reactor. Line 1034 shows the hydrogen Faradaic efficiency of the Piperion reactor. Line 1032 shows the ethylene Faradaic efficiency of the 0.5 wt % THxA reactor. Line 1035 shows hydrogen Faradaic efficiency of the 0.5 wt % THxA reactor. Line 1033 shows the ethylene Faradaic efficiency of the 0.5 wt % OdOH reactor. Line 1036 shows the hydrogen Faradaic efficiency of the 0.5 wt % OdOH reactor.

As seen by the data illustrated in FIG. 10, the coated polyethylene membrane reactors have lower voltages than the standard Piperion AEM reactor while demonstrating the same selectivity for ethylene. Moreover, the data shows that the choice of additive for coating is important in higher concentrations of analyte with the OdOH coating reactor having a less stable voltage over time as compared to the THxA coating indicating that the THxA is less susceptible to degradation during operation.

FIG. 11 illustrates the cell potential and Faradic efficiency for ethylene and dihydrogen conversion of oxocarbon reactors. A first reactor has a Piperion AEM separator. A second

reactor has a polyethylene separator coated with a 0.5 wt % THxA solution. The current density applied to the reactors was 200 mA per centimeter squared of active area on the scale of five centimeters squared. The anolyte in both reactors was 4 M potassium hydroxide. The x-axis of both plots is time in hours. Line 1100 shows the potential voltage across the cell for the Piperion separator. Line 1110 shows the potential voltage across the cell for a 0.5 coating of THxA. Line 1121 shows the ethylene Faradaic efficiency of the Piperion reactor. Line 122 shows the ethylene Faradaic efficiency of the 0.5 wt % THxA reactor. Line 1123 shows the hydrogen Faradaic efficiency of the Piperion reactor. Line 1124 shows the hydrogen Faradaic efficiency of the 0.5 wt % THxA reactor. As seen by the data, a reactor that uses a polyethylene membrane coated with THxA requires lower voltage to achieve a given current density than a reactor that uses a standard Piperion AEM whilst demonstrating the same selectivity for ethylene.

In specific embodiments of the invention, coatings can be applied to separators in various ways. In a first step, the coating chemical can be dissolved in an additive solvent to achieve a desired concentration in wt % of the coating chemical relative to the solvent. The amount of the solvent can be increased to decrease the wt % and the amount of the solvent can be decreased to increase the wt %. In a next step, the separator can be submerged in the resulting solution and allowed to soak for a set period of time such as 24 hours. As used herein, the phrase "a coating having a wt %" can refer to the wt % of the chemical that forms the coating in such a solution. In a next step, the separator can be removed from the solution and placed into activation solution. The separator can be submerged in the activation solution for a set period of time such as 24 hours. In a specific example, a separator formed of polyethylene can be coated with OdOH by dissolving 0.05 grams of OdOH in a mixture of 2 grams of water and 8 grams of propan-2-ol. The polyethylene membrane with a surface area of 16 squared centimeters can then be submerged in the solution for 24 hours. Subsequently, the separator can be removed and placed into a 12-gram solution of 1M potassium hydroxide (KOH) and be left to soak for 24 hours prior to use. The separator can then be dried under a vacuum. In specific embodiments of the invention, the amount of the coating chemical required can be around 0.01 milligrams per centimeter squared of the polyethylene separator. In specific embodiments of the invention, the amount of coating chemical required can be around 0.4 to 3.6 wt % of the dry separator weight.

In specific embodiments of the invention, the separators are thin sheets. The thickness of the separator can be chosen to control the transport rates of species such as anions, cations, and neutral species such as alcohols and water during operation of the electrolysis reactor in which they are installed. Pore size can be selected along with thickness to impact this rate. Generally, for high efficiency reactors faster ionic migration is preferred such that thinner separators are preferred. The sheets can be less than 250 microns ( $\mu$ m) in thickness, may advantageously be less than 200  $\mu$ m in thickness, less than 100  $\mu$ m in thickness, and ideally may be less than 50  $\mu$ m in thickness where the thickness is measured from the anode area to the cathode area. The thinness of the sheet is limited by the mechanical stability of the sheet for a given application and the ability of the sheet to maintain its function as a separator in keeping the chemistries of the anode area and the cathode area separate aside from the allowance of ionic migration across the separator.

In specific embodiments of the invention, the separator is pressed against a cathode area that comprises a catalyst layer

able to reduce a substance (e.g., carbon monoxide or carbon dioxide) to generate value-added hydrocarbons/alcohols/ organic acids or carboxylates. The catalyst can comprise one or more: molecular species, single-metal-site heterogeneous compounds, metal compounds, carbon-based compounds, polymer electrolytes (also referred to as ionomers), metal- organic frameworks, or metal-doped covalent organic frameworks or any other additives. The molecular species can be selected from metal porphyrins, metal phthalocyanines or metal bipyridine complexes. The metal compound can be under the form of metal nanoparticles, nanowires, nano powder, nanoarrays, nanoflakes, nanocubes, dendrites, films, layers, or mesoporous structures. The single-metal- site compounds can comprise a metal-doped carbon-based material or a metal-N—C-based compound. The cathode catalyst may be made of a metal or metal ion from metals such as, but not limited to, Cu, Ag, Au, Zn, Sn, Bi, Ni, Fe, Co, Pd, Ir, Pt, Mn, Re, Ru, La, Tb, Ce, Dy or other lanthanides and mixtures and/or alloys thereof. For example, the cathodic catalyst could comprise Cu such that the electrolyzer assembly included a copper-based cathode. The carbon-based compounds can comprise carbon nanofibers, carbon nanotubes, carbon black, graphite, boron-doped diamond powder, diamond nanopowder, boron nitride or a combination thereof. The additives can be halide-based compounds including F<sup>−</sup>, Br<sup>−</sup>, I<sup>−</sup>, and Cl<sup>−</sup>. The additives can be specifically dedicated to modifying hydrophobicity such as treatment with PTFE or carbon black. The cathode area may further comprise a catalyst layer on a gas diffusion layer, a porous transport layer, or any other support, which encourages the diffusion of the gas from a stream to the surface of the catalyst, as well as allowing the release of non-reacted/product gases. Porous transport layers can also be referred to herein as porous supports.

In specific embodiments of the invention, the separator is pressed against an anode area that comprises an anodic catalyst layer able to oxidize a substance to produce a product and protons/water. The catalyst can comprise one or more: molecular species, single-metal-site heterogeneous compounds, metal compounds, carbon-based compounds, polymer electrolytes (also referred to as ionomers), metal- organic frameworks, metal-doped covalent organic framework, or any other additives. The molecular species can be selected from metal porphyrins, metal phthalocyanines or metal bipyridine complexes. The metal compound can be under the form of metal nanoparticles, nanowires, nano powder, nanoarrays, nanoflakes, nanocubes, dendrites, films, layers, or mesoporous structures. The single-metal- site compounds can comprise a metal-doped carbon-based material or a metal-N—C-based compound. Anodic catalyst species used for this purpose could include, but are not limited to, metals and/or ions of: Ir, Co, Cu, Ni, Fe, Pt, Rh, Re, Ru, Pd, Os, Mo, and mixtures and/or alloys thereof. For example, the anodic catalyst could be Ni such that the electrolyzer assembly included a nickel-based anode. The carbon-based compounds can comprise carbon nanofibers, carbon nanotubes, carbon black, graphite, boron-doped diamond powder, diamond nanopowder, boron nitride or a combination thereof. The additives can be halide-based compounds including F, Br, I, and Cl. The additives can be specifically dedicated to modifying hydrophobicity such as treatment with PTFE or carbon black. The anode area may further comprise a catalyst layer on a gas diffusion layer, a porous transport layer, or any other support, which encourages the diffusion of the gas from a stream to the surface of the catalyst, as well as allowing the release of product gases.

In specific embodiments of the invention, the porous support for either the anode area, the cathode area, or both, can be selected from carbon-based porous supports or metal- based porous material or a combination. The carbon-based porous support can be based on carbon fibers, carbon cloth, carbon felt, carbon fabric, carbon paper, molded graphite laminates and the like or a mixture thereof. The carbon- based porous support can be a gas diffusion layer with or without microporous layer. Such carbon-based support can be in particular chosen in the among the following list: Sigracet 39AA, Sigracet 39BC, Sigracet 39BB, Sigracet 39BA, Sigracet 36AA, Sigracet 36BB, Sigracet 35BC, Sigracet 35BA, Sigracet 29BA, Sigracet 28BB, Sigracet 28AA, Sigracet 28BC, Sigracet 25BC, Sigracet 22BB, Sigracet 35BI, Toray papers, Toray THP-H-030, Toray TGP-H-060, Toray TGP-H-090, Toray TGP-H-120, Freudenberg H23C6, Freudenberg H15C13, Freudenberg H15C14, Freudenberg H14C10, Freudenberg H14CX483, Freudenberg H14CX653, Freudenberg H24CX483, Freudenberg H23C6, Freudenberg H23C8, Freudenberg H24C5, Freudenberg H23C3, Avcarb MB-30, Avcarb GDS5130, Avcarb GDS2130, Avcarb GDS3250, Avcarb GDS3260, Avcarb GDS2230, Avcarb GDS2240, Avcarb GDS2255, Avcarb GDS2185, AvCar 1071, AvCarb 1698, AvCarbon 1209, AvCarb 1185, AvCarb1186, AvCarb 7497, AvCarb T1819, AvCarb T1820, AvCarb T1824, AvCarb 1071, AvCarb 1698, AvCarb 1209, AvCarb 1185, AvCarb 1186, AvCarb 1186, AvCarb T1819, AvCarb T1820, AvCarb T1824, AvCarb EP40, AvCarb P75, AvCarb EP55, AvCarbon EP40T, AvCarb P75T, AvCarb EP55T, AvCarb MGL190, AvCarb MGL280, AvCarbMGL370. The metal-based porous support can be selected from titanium, stainless steel, Ni, Cu, or any other suitable metal and can be under the form of mesh, frit, foam or plate of any thickness or porosity.

In specific embodiments of the electrolyzer, the high mechanical strength of the separator is exploited in the deposition of catalyst layers onto the separator. In these embodiments, the cathode catalyst layer, the anode catalyst layer, or both are applied directly onto the separator through techniques such as reactive spray deposition, ultrasonic spraying, air brushing, brushing, drop-casting, spin coating, electrospinning, or through transfer from an ink-loaded support. The separator may be hot-pressed to encourage interaction between the applied catalysts and the separator.

In specific embodiments of the invention, the system can include an electrolyte that will facilitate the transportation of ions and provide ions that promote the reactions. In some embodiments of the technology, the electrolyte may be an alkaline solution such as a solution of hydroxide-containing salt such as but not limited to potassium, sodium or cesium hydroxide with concentrations such as (0.01 molarity (M), 0.05 M, 0.1 M, 0.2 M, 0.5 M, 1 M, 2 M, 3 M, 4 M, 5 M, 6 M, 7 M, 8 M, 9 M and 10 M). The use of concentrated alkaline solution brings down the energy requirement of the overall reaction. Alkali metal cations (such as Li, Na, K, Cs, and Rb) may be used as counter-cations. In other embodiments of the reactor, the electrolyte may contain salt with cations such as Lit<sup>+</sup>, K<sup>+</sup>, Na<sup>+</sup>, Cs<sup>+</sup>, Rb<sup>+</sup>, Fr<sup>+</sup>, with anions including, but are not limited to HCO<sub>3</sub><sup>−</sup>, CO<sub>3</sub><sup>2−</sup>, Cl<sup>−</sup>, Br<sup>−</sup>, I<sup>−</sup>, OH<sup>−</sup>, ClO<sub>4</sub><sup>−</sup>, IO<sub>4</sub><sup>−</sup>, SO<sub>4</sub><sup>2−</sup>, and NO<sub>3</sub><sup>−</sup>. The anion may be oxidized during electrolysis. Given that the conductivity of the system is determined by the electrolyte, changes to electrolyte composition and concentration has considerable influence on the voltage/current characteristics and selectivity of the device. The electrolyte may be introduced through the anodic chamber, the cathodic chamber or be applied

directly to the separator through a separate inlet. In specific embodiments of the invention, the electrolyzer is used to produce high-added-value products from carbon monoxide, such as but not exclusively, acetate, ethanol, ethylene, propanol, and propionate. The electrolyte in these embodiments can be hydroxide based. In specific embodiments of the invention, the electrolyzer is used to produce high-added-value products from carbon dioxide, such as but not exclusively carbon monoxide, syngas, formic acid, acetic acid, ethanol, ethylene, propanol, and propionate. The electrolyte in this embodiment can be based on an alkali metal carbonate or alkali metal bicarbonate, such as  $K_2CO_3$ ,  $KHCO_3$ ,  $Na_2CO_3$ ,  $NaHCO_3$ ,  $Li_2CO_3$ ,  $LiHCO_3$ ,  $Cs_2CO_3$ ,  $CsHCO_3$  or a mixture thereof.

The electrolyte can be applied to the electrolyzer in various ways. In specific embodiments of the invention, an electrolyte input feeds electrolyte directly to the separator. The electrolyte can be delivered directly to the separator in this example by extending the separator beyond the edges of the reactor cell to which it is a part and allowing electrolyte to be absorbed into the separator through capillary forces. In alternative embodiments of the invention, an electrolyte input flows electrolyte through a cathodic input stream, or an anodic input stream and the electrolyte is applied to the separator via the fact that the separator is in contact with the anode area or cathode area. The electrolyzers can take as an input, a cathodic input stream (e.g., stream enriched in carbon monoxide or dioxide) and an anode input stream. The cathodic input stream can be provided to an inlet connected to the cathode flow field. The anodic input stream can be provided to an inlet connected to an anode flow field. The cathodic stream and anodic stream can flow through the stack from the inlets to the outlets and be distributed through the flow channels to each cathodic and anodic area separately. The anodic stream and cathodic stream can flow through separate channels on either side of the cell. Alternatively, at least one of the cathodic and anodic streams may be provided to each cell individually instead of through a connection crossing all the plates. In this case, each cell has a dedicated fluid inlet and outlet for this cathodic and/or anodic stream. The nature of the anodic stream can be determined by the nature of the targeted oxidation reaction (such as, but not limited to, water oxidation, dihydrogen oxidation, chloride oxidation, halide oxidation, hydrocarbon oxidation, waste organic oxidation). When electrically powered, the carbon oxide electrolyzer carries out the concomitant reduction of carbon oxide and oxidation of the chosen oxidation substrate to produce added-value chemicals such as hydrocarbons, organic acids and/or alcohols and/or N-containing organic products in the output cathodic stream separated from the anodic stream where the oxidation products are specifically collected. For example, the generating of chemicals using carbon oxide and the electrolyzer could involve supplying the volume of carbon oxide to a cathode area of the electrolyzer as a cathodic input fluid and supplying a volume of electrolyte to an anode area of the electrolyzer as an anodic input fluid.

In specific embodiments, the electrolyzer operates with a pressure drop from the cathode to the anode to encourage the diffusion of certain species away from the cathode catalyst layer. In other embodiments the electrolyzer operates at a high absolute pressure to encourage solubilization of substrate carbon oxide gas across the system. The use of a pressure drop across the reactor is advantageous for the following reasons: 1) the gaseous phase of the electrolyzer may be compressed to increase the availability of carbon oxide; 2) the pressure may be used to control the proportion

of liquid water available at the catalytic interfaces; 3) the pressurization can be used to force certain species across the electrolyzer, such as the products of electrolysis or the carbon oxide substrate. The differential pressure can be used to control the presence of liquid water, electrode, and carbon oxide gas at the interface between anode and cathode which may concomitantly lead to superior catalyst selectivity, efficiency, or stability, or all three.

In accordance with specific embodiments of the inventions disclosed herein, the separator has enhanced mechanical stability compared to prior art approaches and is therefore conducive to increased pressure. This allows larger differential pressures to be held across the oxocarbon electrolyzer. This pressure differential may be greater than 200 mbar, may ideally be a greater than 500 mbar pressure differential, and may be greater than 1 bar pressure differential. However, at increasing pressure, the stability of the separator may become too intense of a constraint and limit the flexibility of the design to have an increased number of pores, an increased size of pores, or place a limit on how thin the separator can be made.

FIG. 12 provides a block diagram 1200 of an electrolyzer for reducing carbon dioxide to ethylene, acetate, or other multi-carbon products. In the figure, dotted arrows represent electrochemical conversion and solid arrows represent chemical movement. Block diagram 1200 includes a reactor with a cathode area 1202, an anode area 1203, and a separator 1201 in accordance with the electroneutral porous separators described herein. In this example, the anode area 1203 is aqueous and the cathode area 1202 is gaseous. The reactor includes a pressure differential 1210 with increased pressure on the cathode side. As a result, the pressure pushes against the liquid electrolyte and keeps it from leaking through the separator. The pressure can be tuned to assure that the separator remains saturated with liquid electrolyte while not leaking an unacceptable amount of electrolyte. Furthermore, using the illustrated approach, any electrolyte that does seep through the separator can be recovered and recycled. Block diagram 1200 also includes a gas/liquid separator 1204, a gas/liquid separator 1005, a carbon dioxide separator 1206, and a humidifier 1207. In this example, the technology is used to reduce  $CO_2$  to ethylene while generating a stream of  $O_2$  through the oxidation of  $H_2O/OH^-$ . An alkali metal carbonate electrolyte ( $M_2CO_3$ ) is supplied to the anode and ensures that a good supply of alkali metal cation is present. The cathode is a gas diffusion layer with a catalyst layer of copper particles and the anode is a porous transport layer coated with iridium oxide nanoparticles. The separator 1201 is an electroneutral porous separator in the form of a hydrophilic polytetrafluoroethylene sheet with pores <0.2  $\mu m$  in size and a thickness below 50  $\mu m$ . At the cathode, humidified  $CO_2$  is introduced where it diffuses to the cathode catalyst and is reduced to ethylene (or other multi-carbon products). This reaction is promoted by the presence of the alkali metal cations in the non-charged polymeric separator and produces hydroxide along with the product.



The hydroxide formed subsequently reacts with a second molecule of  $CO_2$  to generate a bicarbonate/carbonate ion:



The generated carbonate may then be removed from the reactor as a stream of concentrated alkali metal carbonate in the cathodic product outlet where it can be separated from the gaseous products.



Alternatively, the carbonate may travel across the non-charged polymeric separator to the anode. At the anode the anodic reaction generates O<sub>2</sub> from the oxidation of water, as well as protons. The production of protons leads to the protonation of the carbonate anions to produce CO<sub>2</sub> and water. The CO<sub>2</sub> and O<sub>2</sub> that form is then released through the anodic chamber.



FIG. 13 provides a block diagram 1300 of an electrolyzer for reducing carbon monoxide to ethylene, acetate, or other multi-carbon products. In the figure, dotted arrows represent electrochemical conversion and solid arrows represent chemical movement. Block diagram 1300 includes a reactor with an anode area 1303, a cathode area 1302, and a separator 1301 in accordance with the electroneutral porous separators described herein. In this example, the anode area 1303 is aqueous and the cathode area is gaseous. Block diagram 1300 includes a gas/liquid separator 1304, a gas/liquid separator 1305, and a carbon monoxide separator 1306. In this example, the electrolyzer is used for the reduction of pure carbon monoxide. The cathode is a gas diffusion layer with a catalyst layer of copper particles and the anode is a nickel porous transport layer. At the cathode, carbon monoxide is introduced where it diffuses to the cathode catalyst and is reduced to ethylene and/or ethanol (or other multi-carbon products). In this example, the electroneutral polymeric separator is a hydrophilic polytetrafluoroethylene sheet with pores <0.2 μm in size and a thickness below 50 μm. This reaction is promoted by the presence of the alkali metal cations in the electrolyte-filled separator and produces hydroxide along with the ethylene and/or acetate.



The hydroxide formed above may be removed from the reactor as a stream of concentrated alkali metal hydroxide in the cathodic product outlet. Otherwise, the hydroxide travels across the electroneutral polymeric separator to the anode. At the anode the anodic reaction generates oxygen gas from the oxidation of water, as well as water. The anodic oxygen gas escapes through the anodic product stream.



The ethylene produced is collected in the gas outlet of the cathodic reactor along with unreacted carbon monoxide. The acetate is either collected in the cathodic compartment as a concentrated alkali metal acetate, or transferred to the anode, where it is collected from the electrolyte. The movement of acetate may be controlled using the pressure drop of the electrolyzer and separator pore size.

FIG. 14 provides a block diagram 1400 of an electrolyzer for reducing carbon monoxide or carbon dioxide to, for example: ethylene, ethanol, propylene, propanol, carbon monoxide or syngas (and potentially other co-products). In the figure, dotted arrows represent electrochemical conversion and solid arrows represent chemical movement. Block diagram 1400 includes a reactor with an anode area 1403, a cathode area 1402, and a separator 1401 in accordance with the electroneutral porous separators described herein and with corresponding water and electrolyte management while introducing the electrolyte through the separator. In this example, the anode area 1403 is aqueous and the cathode area is gaseous. Block diagram 1400 includes a gas/liquid

separator 1404, a gas/liquid separator 1405, an oxocarbon separator 1406, a humidifier 1407, and a gas/liquid separator 1408. In this example, an alkali metal-based salt, or similarly acting alternative, can be used to ensure high ionic conductivity across the cell and is introduced directly into the system through the non-charged polymeric separator. The advantage of this approach is that the flow through the separator may be used to isolate the products crossing the non-charged ionic separator that would otherwise be mixed with products at the anode or cathode. This could be used to mitigate the release of carbon dioxide in the anodic chamber of a carbon dioxide electrolyzer after carbonate acidification:



In this example, the electroneutral polymeric separator is a hydrophilic polytetrafluoroethylene sheet with pores <0.2 μm in size and a thickness below 50 μm. The electrolyte can be delivered directly to the separator in this example by extending the separator beyond the edges of the reactor cell to which it is a part and allowing electrolyte to be absorbed into the separator through capillary forces.

FIG. 15 illustrates a flow chart 1500 for a set of methods for operating an oxocarbon electrolysis reactor comprising several steps. The process includes steps that are conducted prior to operation of the reactor and a set of steps that are conducted simultaneously during operation of the device. Flow chart 1500 includes a step 1501 of separating a cathode area from an anode area using a separator. The step can be conducted using the separators disclosed herein (e.g., electroneutral separators and porous separators).

Flow chart 1500 also includes an optional step 1502 of applying a pressure difference across the oxocarbon electrolysis reactor from the anode area to the cathode area of the reactor. The step can be conducted such that a conductive electrolyte is kept from leaking through the separator. The pressure differential can be controlled to control an amount of electrolyte that is allowed to move through the separator.

Flow chart 1500 continues with an optional step 1503 of applying a conductive electrolyte to the electroneutral separator. If the separator is a porous electroneutral separator, the step can include the electrolyte moving into the pores of the separator. If the separator is a porous electroneutral separator with a porous network, the step can include the conductive electrolyte extending through the electroneutral separator via the porous network. If both optional step 1502 and optional step 1503 are conducted and the separator is a porous separator, optional step 1502 can include the conductive electrolyte being pressed away from the anode area by the pressure difference.

Flow chart 1500 continues with an operational phase of the reactor in which the three illustrated steps occur at the same time. The steps include a step 1504 of reducing an oxocarbon species in a cathode area, a step 1506 of oxidizing an oxidation substrate in an anode area, and a step 1505 of allowing ionic migration between the anode area and cathode area across the electroneutral separator. The steps are conducted simultaneously because it is the ionic migration across the separator that allows the reduction and oxidation reactions to occur in the reactor.

While the specification has been described in detail with respect to specific embodiments of the invention, it will be appreciated that those skilled in the art, upon attaining an understanding of the foregoing, may readily conceive of alterations to, variations of, and equivalents to these embodiments. The disclosure of volumes of chemicals in this disclosure is not meant to refer to a physically isolated

## 25

volume as it is possible for a volume of dihydrogen to exist with a volume of carbon dioxide in a single physical volume in the form of a volume of syngas. Although examples in the disclosure were generally applied to industrial chemical processes, the same approaches are applicable to chemical processing of any scale and scope. Furthermore, while the examples in this disclosure were generally applied to the delivery of carbon monoxide to an electrolyzer, approaches disclosed herein are more broadly applicable to the delivery of any member of the oxocarbon family to an electrolyzer for the purposes of generating useful chemicals therefrom. These and other modifications and variations to the present invention may be practiced by those skilled in the art, without departing from the scope of the present invention, which is more particularly set forth in the appended claims.

What is claimed is:

1. An oxocarbon electrolysis reactor comprising:  
an aqueous anode area with an aqueous oxidation substrate and an electrolyte;  
a gaseous cathode area with an oxocarbon species as a gaseous reduction substrate; and  
an electroneutral separator saturated with the electrolyte, formed of one or more polymers selected from a group consisting of: polytetrafluoroethylene, polyethylene, polypropylene, polystyrenes, polysiloxanes, polyether sulfone, and polyacrylonitrile, and separating the aqueous anode area and the gaseous cathode area while allowing ionic migration between the aqueous anode area and gaseous cathode area, wherein the gaseous reduction substrate is diffused across a cathodic catalyst and the electroneutral separator is pressed against the cathodic catalyst;  
wherein: (i) the electroneutral separator is a polymer having a coating; (ii) the coating is formed of an aliphatic molecule; (iii) the coating increases a hydrophilicity of the electroneutral separator; and (iv) the electroneutral separator is less than 250 microns thick where thickness is measured from the anode area to the cathode area; and (v) the reactor comprises a pressure difference greater than 200 mbar across the oxocarbon electrolysis reactor from the cathode area to the anode area.
2. The oxocarbon electrolysis reactor of claim 1, wherein: the aliphatic molecule is selected from a group consisting of: (i) an aliphatic alcohol; (ii) an aliphatic amine; (iii) an aliphatic ether; (iv) an aliphatic acetal; and (v) an aliphatic ketal.
3. The oxocarbon electrolysis reactor of claim 1, wherein:  
the electroneutral separator is formed of a linear aliphatic carbon chain; and  
the coating is a linear aliphatic carbon chain with a hydrophilic functional group.
4. The oxocarbon electrolysis reactor of claim 3, wherein:  
the electroneutral separator is formed of polyethylene.
5. The oxocarbon electrolysis reactor of claim 4, wherein:  
the coating is selected from a group consisting of: (i) octadecan-1-ol; (ii) trihexylamine; (iii) 2-methylnonadecan-2-ol; (iv) poly (ethylene-co-vinyl alcohol); and (v) poly (ethylene-co-vinyl alcohol) crosslinked with glutaraldehyde.
6. The oxocarbon electrolysis reactor of claim 1, wherein:  
the electroneutral separator is formed of polyacrylonitrile.
7. The oxocarbon electrolysis reactor of claim 1, wherein:  
the electroneutral separator is ionically conductive; and  
the electroneutral separator is formed by electrically insulative material.
8. The oxocarbon electrolysis reactor of claim 1, wherein:  
the electroneutral separator is electroneutral in that no charged chemicals are chemically bound into the electroneutral separator.
9. The oxocarbon electrolysis reactor of claim 1, further comprising:  
a porous network formed by a set of pores and extending through the electroneutral separator.
10. The oxocarbon electrolysis reactor of claim 9, wherein:  
the set of pores is a set of pores each having an average size less than one millimeter.
11. The oxocarbon electrolysis reactor of claim 9, further comprising:  
a conductive electrolyte;  
wherein the conductive electrolyte is an alkaline solution, and the conductive electrolyte extends through the electroneutral separator via the porous network.
12. The oxocarbon electrolysis reactor of claim 9, wherein the electrolyte extends through the electroneutral separator via the porous network and is pressed away from the aqueous anode area by the pressure difference.
13. An oxocarbon electrolysis reactor comprising:  
an aqueous anode area with an aqueous oxidation substrate and an electrolyte;  
a gaseous cathode area with an oxocarbon species as a gaseous reduction substrate;  
an electroneutral separator saturated with the electrolyte, formed of one or more polymers selected from a group consisting of: polytetrafluoroethylene, polyethylene, polypropylene, polystyrenes, polysiloxanes, polyether sulfone, and polyacrylonitrile, and separating the aqueous anode area and the gaseous cathode area while allowing ionic migration between the aqueous anode area and gaseous cathode area, wherein the gaseous reduction substrate is diffused across a cathodic catalyst and the electroneutral separator is pressed against the cathodic catalyst; and  
a porous network formed by a set of pores and extending through the electroneutral separator;  
wherein: (i) the electroneutral separator is a polymer having a coating; and (ii) the polymer comprises aliphatic carbon chains; (iii) the coating is an aliphatic carbon chain with a hydrophilic functional group; and (iv) the electroneutral separator is less than 250 microns thick where thickness is measured from the anode area to the cathode area; and (v) the reactor comprises a pressure difference greater than 200 mbar across the oxocarbon electrolysis reactor from the cathode area to the anode area.
14. The oxocarbon electrolysis reactor of claim 13, wherein:  
the aliphatic carbon chain is formed of a monomer selected from a group consisting of: (i) an aliphatic alcohol; (ii) an aliphatic amine; (iii) an aliphatic ether; (iv) an aliphatic acetal; and (v) an aliphatic ketal.
15. The oxocarbon electrolysis reactor of claim 13, wherein:  
the electroneutral separator is formed of polyethylene.
16. The oxocarbon electrolysis reactor of claim 15, wherein:  
the coating is selected from a group consisting of: (i) octadecan-1-ol; and (ii) trihexylamine; and (iii) 2-methylnonadecan-2-ol; and (iv) poly (ethylene-co-vinyl alcohol); and (v) poly (ethylene-co-vinyl alcohol) crosslinked with glutaraldehyde.

## 26

## 27

17. The oxocarbon electrolysis reactor of claim 13, wherein:

the electroneutral separator is formed of polyacrylonitrile.

18. The oxocarbon electrolysis reactor of claim 13, wherein:

the electroneutral separator is ionically conductive; and the electroneutral separator is formed by electrically insulative material.

19. The oxocarbon electrolysis reactor of claim 13, wherein:

the electroneutral separator is formed by a polymer; and the electroneutral separator is electroneutral in that no charged chemicals are chemically bound into the electroneutral separator.

20. The oxocarbon electrolysis reactor of claim 13, wherein:

the set of pores is a set of pores each having an average size less than one millimeter.

21. The oxocarbon electrolysis reactor of claim 13, further comprising:

a conductive electrolyte;

wherein the conductive electrolyte is an alkaline solution, and the conductive electrolyte extends through the electroneutral separator via the porous network.

22. The oxocarbon electrolysis reactor of claim 13, wherein conductive electrolyte extends through the electroneutral separator via the porous network and is pressed away from the aqueous anode area by the pressure difference.

23. A method of operating an oxocarbon electrolysis reactor comprising:

## 28

reducing an oxocarbon species in a gaseous cathode area; oxidizing an oxidation substrate in an aqueous anode area including an electrolyte;

separating the gaseous cathode area from the aqueous anode area using an electroneutral separator formed of one or more polymers;

allowing ionic migration between the aqueous anode area and gaseous cathode area across the electroneutral separator and selected from a group consisting of: polytetrafluoroethylene, polyethylene, polypropylene, polystyrenes, polysiloxanes, polyether sulfone, and polyacrylonitrile; and

saturating the electroneutral separator with the electrolyte;

wherein: (i) the electroneutral separator is a polymer having a coating; (ii) the polymer comprises aliphatic carbon chains; (iii) the coating is an aliphatic carbon chain with a hydrophilic functional group; (iv) the electroneutral separator is less than 250 microns thick where thickness is measured from the anode area to the cathode area; and (v) the reactor comprises a pressure difference greater than 200 mbar across the oxocarbon electrolysis reactor from the cathode area to the anode area.

24. The method of operating the oxocarbon electrolysis reactor of claim 23, wherein:

the aliphatic carbon chain is formed of a monomer selected from a group consisting of: (i) an aliphatic alcohol; (ii) an aliphatic amine; (iii) an aliphatic ether; (iv) an aliphatic acetal; and (v) an aliphatic ketal.

\* \* \* \* \*